# EUROPEAN PATENT SPECIFICATION

(11) **EP 0 437 672 B1**
(45) Date of publication and mention of the grant of the patent: **08.06.1994**
(21) Application number: 90114902.1
(22) Date of filing: 02.08.1990
(51) Int. Cl.: B28B 1/14

(54) **Method of manufacturing intermediate concrete products, formwork for manufacturing said products, and apparatus for carrying out said method**
Verfahren zur Herstellung von Betonkörpern, Schalung für die Herstellung dieser Betonkörper und Vorrichtung zur Durchführung des Verfahrens
Procédé de production de produits en béton, coffrage pour produire lesdit produits, et appareil pour exécuter ledit procédé

(30) Priority: 16.01.1990 YU 72/90
(43) Date of publication of application: 24.07.1991
(73) Proprietor: ZAVOD ZA RAZISKAVO MATERIALA IN KONSTRUKCIJ, N.SOL.O. TOZD INSTITUT ZA MATERIALE, N.SUB.O., SI-61109 Ljubljana (SI)
(72) Inventor: Korla, Jadran, SI-61000 Ljubljana (SI); Mali, Edvard, SI-64000 Kranj (SI); Gjura Janez, SI-61000 Ljubljana (SI); Spasic, Miroslav, SI-61000 Ljubljana (SI); Bajc, Ivan, SI-61000 Ljubljana (SI); Zajc, Andrej, SI-61000 Ljubljana (SI); Bernik, Mitja, SI-61000 Ljubljana (SI); Pozun, Janez, SI-61000 Ljubljana (SI); Durini, Janez, SI-61000 Ljubljana (SI)
(74) Representative: Viering, Jentschura & Partner

(56) References cited:
- DD-A- 259 576
- GB-A- 1 579 544
- DER GRUNDBAU, Armin SCHOKLITSCH, Verlag Julius Springer, Wien, 1932, pages 118-119
- DIE GRÜNDUNG VON BAUWERKEN, Wolf PLAGEMANN, Wolfgang LANGNER, Verlag B.G. Teubner, Leipzig, 1973, page 106

## Description

The invention refers to a method of manufacturing intermediate concrete products according to the precharacterizing part of claim 1.

In building constructions as roofing tiles made of clay or concrete are used at most. Since in primary sense the production of clay tiles is locally bound to a basic stock of raw material and preferably to greater stationary plants characteristic of a high power consumption on the production spot, there asset themselves more and more concrete tiles which correspond to clay tiles both in form and quality.

The concrete tiles are manufactured according to a known method in such a manner that concrete of dry to damp consistency, having as a rule no additional dyes, is fed onto a horizontal formwork and consolidated into the corresponding form by means of vibrating and compressing. Further, raw tile formed in such a manner proceeds into a heating chamber in which there prevail specified climatic conditions (humidity of 95% and temperature of up to 65 °C) and reposes until it has won approximately 50% of its ultimate strength. Only then the tile can be lifted out of the horizontal formwork and proceeded to further treatment, e.g. sorting, colouring, storage.

Due to technological features of the concrete of dry to damp consistency, there exists at known methods a problem of how to attain good homogeneity and mixing of components of the concrete, particularly those which appear in small quantities (from O,5% to 5% by weight of cement) in a concrete mixture. This problem is particularly obvious in chemical admixtures for improving the persistency of the concrete product and in adding dyes into the concrete mixture. Said problems result in a variable quality of the products both in technological and in visual sense. A disadvantage of the concrete of said consistency is also a relatively high sensitivity to changes of volume in loose and consolidated state, which results in a change of quality of the product even at the slightest changes of input material, e.g. humidity.

A further disadvantage of the known method lies in a high sound pressure level occurring at consolidating the concrete by means of vibrations, due to intensive vibrating of the concrete there also appear powerful vibrations in the surrounding of the tile producing machine. During consolidating the tiles, deformations of the horizontal metal formworks take place, which results in the necessity of frequently replacing the formworks to avoid deformed products.

Another disadvantage of the known method lies in the circumstance that the side of the concrete product-tile facing away from the formwork is free, i.e. unprotected, wherefore damages can occur on the tile. During the time in which the tile lies in the chamber, even the entire surface of the tile which at use is exposed to weather can be damaged due to possible change of humidity or temperature.

A further disadvantage lies in that a great amount of space is needed for the aforementioned method of manufacturing tiles as the daily production of e.g. 100.000 tiles requires approximately 12.000 m³ of room which, in addition, should be heated to a temperature of approximately 65 °C , which results in a relatively high power consumption.

From "Der Grundbau", Armin SCHOKLITSCH, Verlag Julius Springer, Wien, 1932, page 118, line 27 - page 119, line 3; fig. 136b; and from "Die Gründung von Bauwerken", Wolf PLAGEMANN, Wolfgang LANGNER, Verlag B.G.Teubner, Leipzig, 1973, page 106, especially page 106, lines 18-19, fig. 10.10b, it is generally known to build foundation wherein the concrete is fed into a form by a nozzle and the outlet of the nozzle is moved in that way during feeding of the concrete into the form, that the outlet of the nozzle is kept under the surface of the concrete for a certain distance.

Moreover, from the GB-A-1 579 544 generally a box connected to a plurality of tubes is known for feeding concrete into a plurality of casts; and the DD-A-259 576 shows generally a distributor system for liquids, especially chemical agents and pharmaceutical agents.

The object of the invention is to provide a method of manufacturing concrete products, preferably tiles, according to the precharacterizing part of claim 1, in which the aforementioned disadvantages will be avoided.

This object is according to the invention gained by means of features given in the characterizing clause of claim 1. Advantageous embodiments of the invention are defined by the subclaims 2 and 3.

It is understood that the present invention can be used for different intermediate concrete products too, although it is specifically described for concrete tiles.

The invention is further described in the following preferred embodiment, reference being made to the accompanying drawings. Therein show:
Fig. 1 a schematic diagram of an apparatus for carrying out the method according to the invention,
Fig. 2 a side elevation of a charging head of an apparatus for carrying out the method according to the invention,
Fig. 3 a view of the charging head in the direction of an arrow III of Fig. 2,
Fig. 4 a vertical sectional view of the charging head,
Fig. 5 a view in the direction of an arrow V of Fig. 4,
Fig. 6 a detail of a blocking unit in closed position,
Fig. 7 a detail of a blocking unit in open position,
Fig. 8 a plan view of a formwork for manufacturing tiles according to the invention,
Fig. 9 a sectional view of a formwork taken along the line IX-IX of Fig. 8, and
Fig. 10 an element of a formwork according to the invention.

The feature of the present method according to the invention lies in the use of concrete of a cast consistency, which ensures uniformity of the composition and unsegregability of concrete, the possibility of forwarding under pressure to the charging head and filling up a row of formworks during one production cycle with exact material dosing. Cast concrete possesses the features of good and quick homogeneity even in the case when very small quantities of chemical or mineral additives are added. Thus, obtaining high degree of uniform quality, there are ensured the durability of the material, e.g. resistance to freezing and chemical influence resistance and high quality of pigmentizing of concrete mass. Components of the cast concrete ensuring the necessary features of fresh concrete admixture are as follows:
- cement, preferably highly active cement,
- stone aggregate with size gradation of at most 3,2 mm and sifting of 15% to 20% through a 0,25 mm sieve,
- usual chemical admixture for lowering the surface tension of the water,
- usual chemical admixture for introducing microporosity into the cement paste,
- mineral fine-grained admixture for preventing micro-mixing (micro-segregation) of concrete and decreasing permeability of the concrete admixture to water,
- mineral fine-aggregate admixture for volume reduction of concrete mass,
- water, and
- mineral dyes.

The method according to the invention will be further described in detail referring to Fig. 1 showing a schematic diagram of an apparatus for carrying out said method. Concrete of the aforementioned composition and consistency is prepared in a common counterflow concrete plant. Concrete prepared in such a manner is delivered into a storage bin 1 of a screw pump 2, by means of which it is conveyed through a pipe line 3 to a charging head 4 of an apparatus according to the invention. In the given case the charging head 4 is arranged for filling up a row of formworks 5 whereby concrete is contractionally discharged into each formwork 5 by means of discharging nozzles 6. Pressure required for operation of the system is maintained by means of automatic synchronised working of the pump 2 and of the unit for opening and closing the stops and unit for lowering and lifting the head 4, whereby it is particularly important that in all nozzles 6 for filling up the formworks 5 the same pressure is ensured. Its value at the outlet of each nozzle 6 equals from 0,1 bar to 0,5 bar, preferably 0,2 bar. Due to technological features of concrete, said formworks must be water-impermeable and made of thermally insulating material, e.g. polyurethane resin. Each nozzle 6 of the charging head 4 is thrust to the area of the bottom of each formwork 5 and then concrete is conveyed therein.

When the formwork 5 is filled up for essentially one third by the height, the charging head 4 and the nozzles 6 are lifted up with constant velocity till the formworks 5 are completely filled up. The nozzles 6 may not be lifted over the level of the concrete being cast in any case. The lifting velocity of the charging head 4 and thereby of the nozzles 6 is adjusted to the largest cross-section of the product being cast, and in the particular case equals from 0,05 ms⁻¹ to 0,2 ms⁻¹, preferably 0,1 ms⁻¹.

When the formworks 5 are filled up they are transferred to a setting place. As said formworks are made of thermally insulating material an intrinsic energy-hydration heat of the cement is exploited released during setting time for the concrete. In such a manner the concrete is aging practically in adiabatic conditions, and after approximately 24 hours reaches a temperature of approximately 55 °C above ambient temperature, which in the particular case equals 20 °C without additional heating wherefore any further thermal treatment is superfluous.

Figs. 8, 9, 10 show, just for further elucidation of the method according to the invention, a formwork 5 for casting concrete tiles. Said formwork comprises a pair of frames 7, 8 clamping together a plurality of elements 9 made of waterimpermeable and thermally insulating material, e.g. polyurethane resin, the form of which corresponds to a product desired, and in the particular case corresponding to a tile. Each element 9 is along both vertical sides provided with a pair of thickenings 10, 11 whereby facing sides of each thickening 10, 11 of two adjacent elements 9 are parallel abutting slitlessly to each other. The element 9 is at its first, in the particular case its lower, end provided with a web 12 being essentially perpendicular to said element and running between the thickenings 10, 11. In the formwork assembled to a block of elements 9 said web slitlessly rests against the adjacent element 9 forming a bottom 13 of the formwork 5 in the essence. The elements 9 are formed in such a manner that their first flat side 14 corresponds to the first side of the tile, their second flat side 15 corresponding to the second side thereof. In the formwork 5 the elements 9 are arranged vertically, i.e. concrete is cast from the upper side. Two elements 9 are needed to produce one tile and n+1 of said elements are needed to produce n tiles.

Just for further elucidation of the method according to the invention, referring to Figs. 1 to 7, an apparatus for carrying out the method of manufacturing concrete products, preferably tiles,is described. The apparatus comprises a storage bin 1 arranged on a screw pump 2. The latter is driven through a gearbox 2' by means of a drive 2''. A pipe line 3 fixed on a stand 3' is connected to the discharge end of the pump 2. The other end of the pipe line 3 is connected to an essentially trapezoidal charging head 4 to which a row of discharging nozzles 6 is interconnected. Said nozzles are removably fixed to a bottom 7 of the head 4 which is in the area of penetration of each nozzle 6 therethrough provided with a wear resisting plate 8. Sides of the plate 8 facing away from the bottom 7 lie in the plane parallel thereto. A blocking unit 8' is slidingly and movably arranged on the plates 8 of each row of the nozzles 6. Said unit comprises closures 9 being mutually rigidly connected by means of a linkage 10 which is interconnected with the pneumatic or hydraulic working cylinder 11. The latter enables simultaneous moving of all closures 9 over the plates 8 and closing and opening the nozzles 6 respectively.

In the area above each closure 9 there are throttle knives 12 arranged slidingly and movably in the same plane as said closure and extending over the entire length of each row of nozzles 6. The throttle knives 12 are regarding the closure 9 staggered in their plane in the direction away from the working cylinder 11, the closures 9 being provided with a lug 9' cooperating with the knives 12. The side of the knives 12 facing away from the working cylinder 11 is shaped as a half-wave of a sinusoidal curve 13 the curvature of which is conditioned by mutual distance of the two utmost nozzles 6, by material cast and by the pressure for pressing material into the nozzles 6. On their side facing away from the bottom 7 the throttle knives 12 are reinforced by means of a brace fillet 14 and mutually connected by means of a linkage 15. On the linkage 10 there is provided a back stop 16 meshing with the linkage 15. The latter penetrates the wall 4' of the head 4 on the side facing away from the working cylinder 11 whereby the linkage 15 is between the said wall and a limit stop 17 provided with a tension-compression spring 18 which enables moving of the throttle knives 12. To a part of the linkage 15 projecting through the wall 4' a nut 18' is screwed thereon, the stroke of the throttle knives 12 being regulated therewith.

The operation of the blocking unit is further described with reference to Figs. 6 and 7. In the starting position the nozzles 6 are closed by means of closures 9. The lugs 9' arranged on said closures hold the throttle knives 12 in a closed position. Moving the closures 9 by means of the linkage 10 and the working cylinder 11 in the direction towards the cylinder 11 reflects in an opening of the nozzles 6. The spring 18, which is compressed in the starting position, repulses the throttle knives 12 by means of the limit stop 17 and the linkage 15 in the same direction as the closures 9 are moving. The spring 18 acts onto the throttle knives 12 until the nut 18' rests against the wall 4' of the head 4. Thus, the closures 9 continue to move so that they completely open the entrance into the nozzles 6. Between that side of each throttle knife 12 lying in front of the curve 13, and the lug 9' of each closure 9 there is a distance a at nozzles 6 completely open, in dependence upon the material cast. Thus, entries into the nozzles 6 due to curve 13 on the knives 12 overlap in a different degree when the closures 9 are in the open position. The more the entrance of each nozzle 6 lies away from the place of supply of the concrete mass into the charging head 4, the smaller the degree of overlapping. In such a manner the same pressure is ensured at the entrance into each nozzle 6 and, therefore, at the outlet thereof for, the smaller the degree of overlapping, the lower the pressure drop. The degree of overlapping thus represents the function of the mutual distance of the utmost two nozzles 6, of the material cast, and of the pressure for pressing material into the nozzles 6.

The entrance into the nozzles 6 is closed by means of the working cylinder 11 pushing the closures 9 through the linkage 10 and the lug 9' of each closure 9 pushing the throttle knives 12 into the starting position. The spring 18 is therefore compressed and the blocking unit 8' is ready for the next working cycle.

## Claims

1. A method of manufacturing intermediate concrete products, wherein a non-segregable concrete of cast consistency is pressed contractionally through at least one nozzle into at least one corresponding formwork, whereby the nozzle is located in the bottom area of the formwork, and when the latter being filled up for essentially one third by the height the nozzle is lifted up with a constant velocity from the formwork in such a manner that it is not lifted over the level of concrete being cast in any case, characterized in that the formwork ist made of a water-impermeable and thermally insulation material, the concrete is aging practically in adiabatic conditions, and the pressure value of dosing of concrete at the outlet of each nozzle (6) equals from 0,1 bar to 0,5 bar, preferably 0,2 bar.

2. A method according to claim 1, characterized in that the lifting velocity of the nozzles equals from 0,05 ms⁻¹ to 0,2 ms⁻¹, preferably 0,1 ms⁻¹.

3. A method according to claim 1, characterized in that the hydration heat of the cement is exploited released during setting time for the concrete.

## Patentansprüche

1. Verfahren zur Herstellung von Betonkörpern, wobei konsistenter, nicht absonderbarer Gussbeton durch wenigstens eine Düse in wenigstens eine entsprechende Schalung nach dem Contractor-Verfahren gepresst ist, wobei die Düse im Bodenbereich der Schalung angeordnet ist und, falls letztere im wesentlichen bis zu einem Drittel in die Höhe ausgefüllt ist, die Düse mit gleichförmiger Geschwindigkeit aus der Schalung herausgezogen wird, u.z. in solcher Weise, dass sie keinesfalls über die Oberfläche des giessenden Betons gehoben wird, dadurch gekennzeichnet, dass eine Schalung aus einem wasserundurchlässigen und wärmeisolierenden Stoff ausgebildet ist, dass Beton tatsächlich in adiabatischem Zustand abbindet und der Dosierdruck von Beton an einer Ausströmöffnung einer jeweiligen Düse (6) von 0,1 bar bis 0,5 bar, vorzugsweise 0,2 bar, beträgt.

2. Verfahren nach Anspruch 1, dadurch gekennzeichnet, dass die Anhebegeschwindigkeit der Düsen von 0,05 ms⁻¹ bis 0,2 ms⁻¹, vorzugsweise 0,1 ms⁻¹ beträgt.

3. Verfahren nach Anspruch 1, dadurch gekennzeichnet, dass die während der Abbindezeit entbundene Hydrationswärme von Zement ausgebeutet ist.

## Revendications

1. Procédé de fabrication de produits intermédiaires en béton, suivant lequel un béton non ségrégable, suffisamment fluide pour être moulé, est envoyé sous pression à travers au moins un ajutage et au moins un moule correspondant, l'extrémité de l'ajutage étant placé au fond du moule, et lorsque le moule est rempli environ au tiers de sa hauteur, l'ajutage est remonté avec une vitesse constante sans que son extrémité ne dépasse en aucun cas la surface du béton, **caractérisé en ce que** le moule est fait d'un matériau imperméable à l'eau et isolant de la chaleur, de manière à ce que la prise du béton s'effectue dans des conditions pratiquement adiabatiques, la pression du béton distribué à l'extrémité de l'ajutage étant comprise entre 0,1 et 0,5 bar et de préférence égale à 0,2 bar.

2. Procédé selon la revendication 1 **caractérisé en ce que** la vitesse d'élévation des ajutages doit être comprise entre 0,005 m.s⁻¹ et 0,2 m.s⁻¹, et de préférence égale à 0,1 m.s⁻¹.

3. Procédé selon la revendication 1 **caractérisé en ce que** la chaleur dégagée par l'hydratation du ciment est utilisée pour favoriser la prise du béton.
